

June 25, 1929.

W. F. BLEECKER

1,718,626

PROCESS OF PREPARING LUMINOUS SURFACES

Filed Oct. 9, 1922



Fig. 1



Fig. 2



Fig. 4



Fig. 3

INVENTOR.  
W. F. BLEECKER

BY  
J. J. DeLannis  
ATTORNEY.

## UNITED STATES PATENT OFFICE.

WARREN F. BLEECKER, OF BOULDER, COLORADO.

## PROCESS OF PREPARING LUMINOUS SURFACES.

Application filed October 9, 1922. Serial No. 593,479.

My invention relates to a process of preparing luminous surfaces and its principal object is to provide a method of applying radio-active and radio-receptive substances to a surface, which produces a high degree of luminosity of the surface in ratio to the superficial extent thereof, at a minimum expenditure of radium compound.

It is well known that in the methods here-  
10 tofore employed in preparing surfaces with substances adapted to emanate light rays, a radio-active compound is intermixed with or adheres to the radio-responsive material in such a manner that but a comparatively small part thereof is exposed for the radia-  
15 tion of light. If, for example, the radio-  
responsive substance with the thereto ad-  
hering radio-active particles is intermixed with a varnish or other similar adhesive, to  
20 form a liquid or semi-liquid paint, the crys-  
tals of the radio responsive substance are  
covered over their entire extent, and when  
the surface to be rendered luminous, is coated  
25 with the mixture, only the radium on the  
exposed surfaces of the outer stratum of the  
granules is capable of emanating its rays,  
while that on the underside of the outer par-  
ticles or that on the crystals which are cov-  
30 ered by the outer layer, is prevented from  
adding to the luminosity of the surface and  
is consequently wasted. In another prior  
method of coating surfaces to render them  
luminous, the surface is, for example, first  
35 covered with the radio-responsive material  
which in turn is covered en masse with the  
radio-active material in pulverulent form.  
It is practically impossible in this method to  
so apply the radium dust that each particle  
is separately exposed at the surface and a  
40 waste of valuable material is again unavoid-  
able. Moreover, in each of the two processes,  
a smooth coating is produced so that the  
luminosity of the exposed self-luminous ma-  
terial is limited by the superficial area of  
45 the surface to which it is applied.

In the process of preparing a luminous surface according to the present invention, all waste of the kind above referred to is avoided and the luminous extent of the surface per unit area, is moreover increased, by first applying the crystalline radio-respon-  
50 sive material in a dry state to the surface,  
and then coating the exposed faces of its  
particles with a radium compound in solu-  
tion. It will be evident that the crystals of

the radio-receptive substance thus applied, present an irregular surface the area of which exceeds the superficial extent of the surface to which it adheres, and that by applying the radium in solution, it is affixed to the exposed 60 faces of the crystals in a thin film of uniform thickness which precludes the waste encountered in other methods as stated hereinbefore.

In carrying out my invention, for exam-  
ple, I paint the surface or design to be made  
luminous, with a thin coating of varnish  
or other glutinous material, cover the wet  
surface with a coating of granular zinc sul-  
fide or other radio-responsive substance in 70  
crystalline form, by dusting, blowing, press-  
ing or other similar method, remove the sur-  
plus sulfide after the varnish has dried, and  
finally coat the exposed surfaces of the crys-  
tals adhering to the varnish, with a neutral 75  
or nearly neutral solution of radium salt such  
as radium chloride, radium bromide, etc., that  
does not dissolve the responsive crystals or  
substance.

It will be apparent from the above de-  
scription that my process has another val-  
uable advantage over other methods in that  
it permits of the application of the radio-  
active and radio-responsive substances, one  
upon the other, in any desired design, since 85  
the glutinous substance can be applied to the  
surface by means of a brush, printing press,  
stamping press or any other known method  
of making or impressing pictorial, typog-  
raphical or other representations upon a sur- 90  
face.

In the accompanying drawing, I have  
shown in Figure 1 a letter rendered luminous  
by my process;

Figure 2, represents a portion of the face of 95  
the letter drawn to an exaggerated scale;

Figure 3, a still further magnified section  
taken on the line 3—3, Figure 2; and

Figure 4, a still further magnified section  
showing the distribution of the radio-active 100  
material upon the crystals of the radio-re-  
sponsive material.

The reference character 2 designates the  
object to which the materials are applied, 3 is  
the glutinous coating, 4 the zinc sulfide crys-  
tals adhering to the coating, and 5 the film of  
radium compound applied in solution, to the  
crystals.

It will be observed that the total extent of  
the radio-active film covering the angularly 110

disposed faces of the exposed portions of the crystals, is far in excess of the superficial area of the design to which the coating is applied and that the luminosity of the design is correspondingly increased. It will furthermore be apparent that inasmuch as the sulfide crystals adhere to the glutinous coating, contiguous to each other, only their exposed faces can receive the film of radio-active solution and that each particle of the radium compound thus applied is continuously active in emanating its alpha rays.

I desire it understood that within the spirit of my invention any radio-responsive material in crystalline form, such as the sulfides of zinc, barium, calcium or strontium, artificial willemite, or others, and any radio-active excitant, such as salts of radium, actinium, ionium, mesothonium, uranium or others, may be employed with varying results and that any glue, varnish or other rapidly drying liquid adhesive is suitable to coat the surface to be rendered luminous.

In the drawings, the crystals of the radio-responsive material have been represented as those of zinc sulfide.

I regulate the predetermined degree of luminosity of the coated surface by varying or establishing the strength of the radium solution. I have found that for all ordinary purposes, a solution of forty micrograms of radium element in one cubic centimeter of water or other suitable solvent, is sufficient to give luminosity equal to that now provided in commercial use, as in watch figures and hands, or to render other articles luminous.

After a design has been rendered self-luminous by my process, its surface may be made more durable by treating it with a soluble sulfate to render insoluble the radium in place, as radium sulfate, which is insoluble in water. The radium-covered surface of the design may also be protected by a thin coating of transparent varnish or it may be covered with glass or other similar transparent material.

I desire it understood that the drawings are merely intended to illustrate the process and that I do not limit myself to the particular embodiments of my invention therein shown and hereinbefore described.

What I claim and desire to secure by Letters Patent is:

1. The method of preparing a luminous surface, consisting in first coating the surface with an adhesive, applying a radio-responsive substance to the adhesive, and covering said substance with a radio-active material in solution. 55

2. The method of preparing a luminous surface, consisting in first coating the surface with an adhesive, applying a radio-responsive substance to the adhesive and covering said substance with a radium compound in solution. 60

3. The method of preparing a luminous 65 surface, consisting in first coating the surface with an adhesive, applying a radio-responsive substance to the adhesive, covering said substance with a radio-active material in solution, and finally treating the material 70 with a soluble sulfate.

4. The method of preparing a luminous surface consisting in covering a radio-responsive material on the surface, with a film of 75 radio-active material in solution.

5. The method of preparing a luminous surface consisting in covering a radio-responsive material on the surface, with a film of 80 radio-active material in solution, and then rendering the radio-active material insoluble. 85

6. The method of preparing a luminous surface consisting in covering a radio-responsive material on the surface, with a film of radio-active material in solution, and then coating 90 said film with a transparent substance. 85

7. The method of preparing a luminous surface consisting in covering a radio-responsive material on the surface, with a film of 95 radio-active material in solution, then rendering the radio-active material insoluble and finally applying a protective transparent covering to the film.

8. The method of preparing a luminous surface, consisting in covering a radio-responsive material on the surface, with a film of radio-active material in solution, and then coating said film with a soluble sulfate. 95

In testimony whereof I have affixed my signature.

WARREN F. BLEECKER.